

June 23, 1942.

V. W. CARPENTER ET AL

2,287,467

PROCESS OF PRODUCING SILICON STEEL

Filed Jan. 3, 1940

2 Sheets-Sheet 1



FIG. 1.

Effect of Dew Point of Hydrogen on Decarburization.  
Open Annealed at 1600° F. for 3 Minutes.  
Thickness .014"



FIG. 2.

Effect of Temperature on Decarburization in Wet Hydrogen.  
Dew Point 130° F.  
Thickness .014"  
Open Annealed for 3 Minutes

INVENTORS.  
VICTOR W. CARPENTER,  
AND JOHN M. JACKSON.  
BY *Allen & Allen*  
ATTORNEYS.

June 23, 1942.

V. W. CARPENTER ET AL

2,287,467

PROCESS OF PRODUCING SILICON STEEL

Filed Jan. 3, 1940

2 Sheets-Sheet 2



**FIG. 3.**

Decarburization Versus Time  
Decarburization at 1500° F. with a Dew  
Point of 130° F.  
Thickness .014"



**FIG. 4.** Time 3 MIN.  
Initial Carbon .05



**FIG. 5.** Time 3 MIN.  
Gage .014 in.



**FIG. 6.** Final Carbon .01  
Temp. 1500° F.



**FIG. 7.** Temp. 1500° F.  
Initial Carbon .05

INVENTORS.

BY VICTOR W. CARPENTER,  
AND JOHN M. JACKSON.

*Allen & Allen*

ATTORNEYS.

## UNITED STATES PATENT OFFICE

2,287,467

## PROCESS OF PRODUCING SILICON STEEL

Victor W. Carpenter, Middletown, and John M. Jackson, Franklin, Ohio, assignors to The American Rolling Mill Company, Middletown, Ohio, a corporation of Ohio

Application January 3, 1940, Serial No. 312,258

12 Claims. (Cl. 148—12)

Our invention relates to decarburization, and though not limited thereto, finds a large field of utility in the production of silicon steel for magnetic purposes, which silicon steel is low in carbon; and we shall describe it principally in connection therewith.

It has long been ascertained that low carbon silicon steel has very many advantages for magnetic uses; but there are a number of manufacturing difficulties connected with the securing of low carbon contents in materials of this class. Theoretically there should be three methods of securing silicon steel sheet or strip containing a minimum of carbon: First, if low carbon silicon steel ingots are made by special melting practice such as induction furnace melting, it should not be necessary to apply to silicon steel sheet or strip either in finished form or in the process of manufacture any treatment for the reduction of carbon. While it is possible to manufacture low carbon silicon steel ingots, and although practices in this connection will likely be improved, yet at the present time it is difficult to get carbon values as low as 0.015 per cent even in small experimental furnaces, and the application of such methods to the large scale, economical production of silicon steel has not yet been accomplished. Second, it is possible to give an intermediate treatment to silicon steel materials in the course of their manufacture into sheet or strip. As set forth in the copending applications of Victor W. Carpenter Serial No. 60,347, filed January 22, 1936, and Serial No. 106,372, filed October 19, 1936, it is a regular commercial practice with certain grades of silicon steel to hot roll to an intermediate gauge and then box anneal the coiled hot-rolled material with the hot mill scale on it at a temperature of between 1350 degrees and 1450 degrees F., substantially cold rolling the material and giving it the necessary heat treatments for magnetic properties. Third, it should theoretically be possible to box anneal the finished sheets in dry hydrogen and secure satisfactory decarburization.

It will be evident that where cold rolling is relied upon to reduce the material to final gauge, it will not be possible to follow a procedure analogous to the second mentioned method but carried on upon the intermediate or finished sheets, because of the absence of the mill scale or any equivalent decarburizing medium. So far as we are aware, prior to the work set forth in this application attempts to decarburize finished cold-rolled silicon steel sheet or strip have not progressed beyond the experimental stage. It is

possible to reduce carbon in silicon steel as low as 0.004 to 0.008 per cent by laboratory box annealing at around 2200° F. for many hours, in dry hydrogen, where the material is in narrow widths, say one or two inches; but as yet we have found no cycle for commercial material which consistently gives low carbon values in the middle portion of wide widths, say sheets or strips 20 to 36 inches wide, other than the process of the present invention.

It may be set forth, therefore, as a fundamental object of this invention that we provide a method of successfully and uniformly decarburizing silicon steel sheet or strip in commercial widths at intermediate or final gages without the necessity of the presence of oxide scale. By the term "decarburization" as hereinafter employed, we mean a substantial per cent reduction of the carbon content to a final value which will depend on the desired properties of the final product and which will always be below 0.015% and often as low as 0.008% or less. This, it will be understood, often amounts to a very considerable decrease in carbon content since the most common commercial melting practices secure silicon steels having carbon contents around 0.04 to 0.06%. It is to be understood, however, that our new process is effective on silicon steels of lower carbon contents and we have, for example, successfully decarburized 0.02% carbon material to a final value of 0.006%.

But it is a further object of our invention to simplify, cheapen and cut down the time duration of a decarburizing treatment carried on on finished sheets or strips. In particular, in the practice of our invention we are able to decarburize these materials during a simple heat treatment of a very few minutes duration and of a character known as open annealing. As a consequence, it is a further object of our invention to provide a decarburizing treatment in the nature of an open anneal, preferably, though not necessarily, continuous, and to provide certain processes of producing silicon steel sheet or strip of very low carbon content and good magnetic properties, which processes do not involve a box anneal.

A further object of our invention is to provide an inexpensive and reliable method of decarburizing cold-rolled material at intermediate or final gages to such an extent that excellent magnetic properties can be produced in wide widths by box annealing in a hydrogenous atmosphere in a commercial length of time.

55 A further object of our invention is to provide

a rapid and practical method of decarburizing relatively narrow strips or sheets or punchings during a batch anneal in piles or coils in which the width of the material is not so great as to prevent the effective access of the annealing atmosphere.

In the preferred practice of our invention we have found that when we operate under certain conditions hereinafter set forth, and heat treat the material in a wet reducing atmosphere we are able to attain the objects of our invention. By way of example in a certain procedure we reduce the carbon content of a silicon steel from its original value of say around 0.04 per cent to not more than 0.008 per cent within three minutes by open annealing the material in wet hydrogen, providing the proper conditions are set up.

The objects of our invention which have been pointed out hereinabove or will be apparent to one skilled in the art upon reading these specifications, we accomplish by that certain procedure of which we shall now describe certain exemplary embodiments with the conditions surrounding them.

Reference is made to the drawings wherein we have charted the variable conditions susceptible of such a showing in the case where the reducing gas is wet hydrogen, and wherein:

Figure 1 is a graph showing the effect of the dew point of the hydrogen used in the open anneal on three classes of materials where the conditions of temperature, time and gauge remain the same.

Fig. 2 is a graph for the same materials showing the effect of temperature variation where the other conditions including the dew point of the hydrogen atmosphere remain the same.

Fig. 3 is a graph showing the effect of time on decarburization in our process where temperature, dew point and gauge remain the same.

Fig. 4 is a solid diagram in which temperature, gauge and final carbon content are plotted against each other, the dew point remaining constant at around 130° F. (15 per cent water vapor by volume).

Fig. 5 is a solid diagram in which initial carbon, final carbon and the annealing temperature are plotted against each other, the dew point remaining constant at around 130° F. (15 per cent water vapor by volume).

Fig. 6 is a solid diagram in which initial carbon, gauge and time are plotted against each other, the dew point remaining constant at around 130° F. (15 per cent water vapor by volume).

Fig. 7 is a solid diagram in which final carbon, gauge and time are plotted against each other, the dew point remaining constant at around 130° F. (15 per cent water vapor by volume).

In the diagrams which form the drawings of this specification legends have been employed so that index numerals are not used. By initial carbon is meant the carbon content of the silicon steel sheet or strip material prior to the decarburizing treatment, while final carbon refers to its content after that treatment.

These diagrams were chosen as exemplary and have to do with the specific determination which form Figs. 1 to 3 inclusive; but they are not limitations upon our invention, our invention being applicable as hereinafter indicated, to all commercial grades of silicon steel containing up to approximately 4 per cent silicon. They are to be regarded primarily as illustrations of how the variables are related so that a skilled worker

may readily apply the process to the material at hand.

As has been indicated, our preferred process involves an open annealing in wet reducing gas such as hydrogen of a certain dew point, for a certain time and at a certain temperature. We shall now proceed to a discussion of the various factors involved. As has been pointed out, pure, dry hydrogen is an exceedingly slow and uncommercial decarburizing medium at any feasible temperature. Wet hydrogen is effective and rapid as we shall hereinafter more fully point out; but we believe that the active decarburizer in our preferred medium is the moisture content, and that the primary function of the reducing gas is to prevent oxidation. For example, we have found that an atmosphere of steam will decarburize quite rapidly; but the tendency to produce oxidation of the sheet somewhat limits its utility as will be understood. A reducing gas permits the decarburizing action but prevents oxidation. We have found in corroboration of this that the optimum of reducing gas will vary with its composition, with the moisture content, and with the temperature. From a metallurgical standpoint it would be desirable to use an atmosphere containing nothing but hydrogen and water vapor; but from an economical standpoint it is frequently desirable to replace part of the hydrogen with nitrogen as occurs when dissociated ammonia is used; or it may be desirable to use as a reducing atmosphere such gases as are commonly produced by the controlled combustion of natural gas. There is, as a consequence, a large permissible variation of the composition of the reducing gas of our preferred atmosphere; and this variation will be dictated by commercial expediency. For best decarburization, however, atmospheres containing high percentages of carbon bearing gases should be avoided.

The mechanism by which carbon is removed from the sheet or strip material is not known. A possible explanation is that either atomic oxygen or atomic hydrogen, or both, derived from the water vapor, is responsible for the rapid rate of decarburization. While we do not desire to be bound by theory, our present feeling is that the water vapor decomposes at the surface of the sheet or strip under the temperature conditions which are maintained and that there ensues a preferential oxidation of the carbon in the presence of both iron and silicon.

The percentage of water vapor in the atmosphere has a very important part in the process of decarburization. At low percentages, for example, one per cent by volume, the rate of carbon removal is very slow; but when the reducing atmosphere contains four per cent or more of water vapor the rate of decarburization becomes quite rapid. This is illustrated in Fig. 1 for certain exemplary analyses of material in an atmosphere of wet hydrogen. Moreover, as the percent of water vapor is increased therebeyond, the rate of decarburization increases, but not as rapidly. It will be noted from Fig. 1 that at 15 per cent of water vapor in the hydrogen the rate of decarburization is still increasing slowly; but it will likewise be clear that the gain in rate by increasing the water vapor content beyond this point is very slow.

There is no maximum water vapor content for decarburization, the only limitation being a practical one that it should not be so high that the material will be objectionably scaled in the atmosphere employed. The concentration of water

vapor which will cause scaling will vary with the temperature, the material and the composition of the balance of the atmosphere in a manner well within the capability of those skilled in the art to determine in the light of these teachings. For example, in an atmosphere composed essentially of hydrogen at 1600° F., it should be permissible to use up to 35% water vapor by volume without scaling most steels. For rapid decarburization water vapor contents should not be used which are below substantially 2 per cent by volume.

The best decarburizing temperatures for commercial open annealing, we have found lie approximately between 1400 and 1600° F. As shown in Figs. 4 and 5 the decarburization in a given time is substantially smaller both above and below this range. While very good results are obtained anywhere within this range on commercial silicon grades, the optimum in decarburization will vary somewhat with the silicon content of the material as hereinafter described. The decarburization in the ranges between 1350 and 1400° F. and between 1600 and 1650° F. is also substantial and will be satisfactory for some applications.

In the batch annealing in wet hydrogen of stacks or coils of relatively narrow material, temperatures still lower than 1350° F. and even as low as 1200° F. will produce effective decarburization although the annealing time will have to be somewhat lengthened. In this type of anneal, however, a decarburizing period of a few hours or more is not commercially objectionable.

The time required for decarburization will depend to a considerable degree upon the gauge of the material used. Three minutes was found to be sufficient (all other conditions being proper) when the material was 0.014 inch thick. From the slope of the curves in Fig. 3 it will be clear that, all other conditions remaining the same, it would require an anneal of approximately 14 minutes to reduce the carbon in a material 0.025 inch thick to as low a value as was obtained with a three minute anneal of material of the same analysis having a gauge of 0.014 inch. In Figs. 6 and 7, gauge appears as one of the variables and these diagrams will give the conditions to be expected over a range broad enough to take care of most commercial requirements.

The effect of the silicon content of materials ordinarily classified as silicon steel on the rate of decarburization seems to be of much less importance. We have noted that when the percentage of water vapor in hydrogen is less than four per cent by volume the higher grades of silicon steel, silicon steels containing the larger commercial quantities of silicon, decarburized at a slower rate, gauge for gauge, than the lower silicon grades. But on the other hand, if the percentage of water vapor is increased to about eight per cent or more, this effect of silicon is not so pronounced. There are indications that as the silicon content increases the optimum decarburizing temperature decreases somewhat. However, with steels containing substantially over 4 percent silicon the rate of decarburization has been found to be so slow that the commercial applications of the process become limited.

But the presence of some silicon is very important to this method of decarburization. While materials substantially or entirely free from silicon may be decarburized, yet the presence of silicon even in very minor quantities, such as a small fraction of one percent, speeds up the de-

carburization. Thus iron and mild steels in general may readily be decarburized by this method if a small percentage of silicon is included in their analyses; and this makes possible the commercial production of very low carbon materials of classes usually not included in the term "electrical steels," or "silicon steels," where the term is used to imply materials of relatively higher silicon contents intended primarily for magnetic uses. Therefore where herein and in the claims which follow, we refer to "silicon steel" without other qualification, we desire to be understood as including also ferrous materials containing sufficient silicon for commercial decarburization by our method, but below the silicon content ordinarily implied by the term "silicon steel." Specifically we desire to be understood as including ferrous materials in which only sufficient silicon has been incorporated to make decarburization commercially feasible, and in general down to substantially 0.05 per cent.

So far as carbon is concerned, naturally the lower the initial carbon the more readily and rapidly can the material be carried down to a specific carbon content set up as a desired standard. In the lighter gauges such as 29 gauge it is not necessary to have the carbon content lower than is normally contained in open hearth heats, in order to accomplish successful decarburization within the exceedingly brief times indicated in our several figures. For heavier gauges, such as 24 gauge, the same time cycles can be achieved if the initial carbon is in the neighborhood of 0.02 per cent. Figs. 5 and 6 show the effect of initial carbon under varying conditions. It will be understood, of course, that our method of decarburization may be practiced upon materials previously partially decarburized by other methods.

Wherever we have referred to an open anneal, we mean the carrying of single or spaced multiple strips or single sheets of material through an elongated heating chamber in which the entire surface of the material has free access to the surrounding annealing atmosphere. This is in distinction to a so-called box anneal in which a tightly wound coil or a large stack of relatively wide sheets is heated to and cooled from the annealing temperature in such a manner that the annealing atmosphere does not have free and uniform access to the entire surface of the material. The temperature is maintained within the preferred range by any suitable heating means in current use in such furnaces, excepting, of course, such heating means as would interfere with the maintenance of the necessary atmosphere. Electric heat and heat applied by means of radiant tubes are, of course, types of heating means which permit great flexibility in the control of atmosphere. Individual sheets may be carried through the furnace on known heat-resisting driven conveyor systems or the sheets may be stitched or otherwise fastened together so as to form the equivalent of a strip. A strip material may be pulled through the furnace in ways current in the art. Although it is theoretically possible to do so, we have not attempted to employ recirculation in connection with the maintenance of the furnace atmosphere. We introduce into the furnace hydrogen or a suitable reducing atmosphere continuously in such volume as to keep oxidizing atmosphere out of the furnace. As a consequence, some of the hydrogen or other reducing atmosphere escapes

at the ends of the furnace where it is burned or carried out a stack.

By following this decarburizing procedure involving the use of wet hydrogen, it is also commercially possible to decarburize silicon steel during a batch anneal in piles or coils in which the width of the material is not so great as to prevent the effective access of the annealing atmosphere. For example, we have found this method successful in decarburizing stacks of 4 inch wide pieces of a 0.014 inch thickness such as are used in transformer cores. Such a decarburizing anneal may be in addition to the final high temperature anneal, or it may be made a part of the regular high temperature anneal by providing the wet hydrogen when the charge is within the correct temperature range and maintaining the temperature of the charge within this range for an effective length of time. This is preferably done during the heating period of the anneal which is then followed by the higher temperature portion of the anneal, which may be, for example, in an atmosphere of dry hydrogen at approximately 2200 degrees F.

The moisture content of the reducing atmosphere may be derived in several ways: We have followed the practice of bubbling the gas through a water bath at a proper temperature to give the desired dew point. We have also admitted controlled quantities of steam to the interior of the furnace when required to maintain a proper dew point. Dew point tests are conducted from time to time and the atmosphere in the furnace is held at the required water vapor content, say between two and thirty-five per cent by volume in ways which will be sufficiently understood by the skilled worker in the art.

Now the provision of a brief open annealing operation which is effective in decarburization renders it possible for us to produce certain grades of silicon steel strip or sheet materials for magnetic uses without the necessity for any box annealing; and further in this connection, it will be observed that the decarburizing anneal can, if desired, be used as the anneal or one of the anneals relied upon for producing the desired magnetic properties.

There are other cases where in order to obtain the best magnetic properties it is necessary to produce a very low carbon material and it is further necessary that the material be box annealed. As has been mentioned, it is practically impossible to decarburize commercial widths of cold-rolled material during the final box annealing. In these cases an intermediate or final decarburization in accordance with our teachings may be desirable in addition to the regular final box anneal. Processes of reducing and treating silicon steel will vary both with the analysis of the steel and with the final result desired, as will be readily understood by the skilled worker in the art. By way of example, a procedure which will produce a silicon steel material characterized by substantially isotropic magnetic properties will differ from a process producing a silicon steel having extraordinary permeability in the rolling direction and very much lower permeability in other directions. The various useful commercial properties in silicon steel for magnetic uses may, however, be secured by combining our new process of decarburization with combinations of processing steps now used. The advantages of these novel combinations will include in some cases lower production costs, in others the production of superior magnetic mate-

rials, in others superior physical properties, and in still others the attainment of excellent magnetic properties which have hitherto been impossible to produce in wide sheets. We give below three exemplary processes falling within the scope of our invention.

In the first process we hot roll the silicon steel to the most economical hot-rolled thickness. Next we pickle it to remove the hot-mill scale and fit the material for cold rolling. Next we cold roll the material to within five to ten per cent of the final gauge, depending upon the silicon content. Next we open anneal the material in wet hydrogen at 1400 to 1600 degrees F. or thereabouts. This step constitutes not only a decarburizing treatment but is also the necessary anneal following the initial cold rolling. Next we cold roll the material to final gauge which will amount to a critical straining of the material by a reduction of five to ten per cent. A final open anneal is given to the material at 1500 degrees F. or higher, depending upon the magnetic quality desired and the silicon content. Wet hydrogen may also be used for this anneal, if desired.

A simpler process not involving critical straining is as follows: Hot roll silicon steel material to the most economical thickness; pickle it preparatory to cold rolling; cold roll it to gauge and then open anneal it so that it is at 1500 degrees F. or thereabouts, in wet hydrogen for at least a portion of the annealing cycle. The final annealing thus not only constitutes the carbon removal but also is the final anneal for developing the desired properties.

In the production of a material characterized by extraordinary permeability in the rolling direction, the following procedure is carried on (it being understood that the gauges given are exemplary only and are intended to indicate proportional relationships): Hot roll the material to say 0.120 inch; box anneal the material for the sake of uniformity in results in the subsequent steps; cold roll to say 0.025 inch with such control of the temperature as will result in an incipient twinned condition of the crystals; open anneal it so that it is at 1500 degrees F. or thereabouts in wet hydrogen for at least a portion of the annealing cycle (which not only decarburizes but constitutes the necessary annealing following the first cold rolling) so that the twinned condition of the crystals can grow by accretion; then cold roll to a final thickness of say 0.012 inch with temperature control and then open anneal so that in the final product the crystal orientation in the silicon steel is preponderantly of the twin-derivative type. This annealing again may be an annealing in wet hydrogen, if desired. A final box anneal may then be added or may replace this last open anneal. We have found that the cold reduction at the first cold rolling stage should be between substantially 60 per cent to substantially 85 per cent, and at the second cold-rolling stage, between substantially 50 per cent and substantially 85 per cent. The initial box anneal, if carried on in the presence of the hot mill scale will effect a partial decarburization of the material. Another alternative in this process is to use an ordinary open anneal at the intermediate gauge and decarburize in wet hydrogen only at the final gauge. It is to be understood that the specific gauges cited are only exemplary; and while they represent a preferred procedure, are not limitations of the process, since, for example, hot rolled starting

materials varying in gauge from 0.07 to 0.15 inch have been effectively used.

This process as here briefly outlined is a modification, in accordance with our present invention, of the processes set forth and claimed in Patent No. 2,158,065 to Cole and Davidson, issued May 16, 1939, and the copending application of Cole, Davidson and Carpenter, Serial No. 235,098, filed October 14, 1938, and the control referred to above is the control set forth in the said patent and application.

The twin-derivative type of crystal orientation mentioned in this process is one in which a preponderance of the crystals are aligned so that a (100) direction is substantially parallel to the rolling direction of the sheet and a (110) plane substantially parallel to the sheet surface.

The inclusion of our new step of decarburization in these processes has resulted in our being able consistently to produce material in wide sheets which, in addition to high-induction permeability, have extremely low core loss. Heretofore it has been impossible consistently to produce wide sheets having extremely low core loss because of the difficulty of eliminating carbon from the centers of wide sheets during the final box annealing in a hydrogenous atmosphere. The value of this new decarburization method to this particular process will at once be apparent.

In any of the above examples of cold-rolling processes involving wet hydrogen decarburization at intermediate or final gauges, under circumstances where it is desired to insure that the finished material will have a very low carbon content, such as 0.003 to 0.008 per cent, it may be commercially advantageous to introduce a decarburizing box anneal at 1200 to 1700 degrees F. for two to twenty-four hours of the unpickled, hot-rolled material prior to the cold rolling. In those processes already having a box anneal at this stage such a decarburizing box anneal can be substituted. By a "decarburizing box anneal" we mean a box anneal in the presence of the hot-mill scale, or its equivalent.

The wet hydrogen decarburizing process can effectively be introduced at other stages in the processing than those of the above examples. For example it may be used following a final high-temperature anneal if the surface of the material is sufficiently clean. Any stage at which the gauge is sufficiently thin so as not to require a non-commercial length of time and at which the surface of the material is sufficiently clean will be satisfactory. The preferred condition is a cold-rolled surface or a surface cleaned by pickling or an equivalent surface. The presence of scale or reduced scale should be avoided.

While this decarburizing process has been described in its particular application to cold-rolled material, it is to be understood that it is also applicable to hot-rolled material. The same teachings as to gauge, carbon content, silicon content, moisture content, and surface condition are directly applicable.

Modifications may be made in our invention without departing from the spirit of it. We have set forth hereinabove the varying factors covering both decarburization per se in accordance with our invention and procedures involving such a step.

Having thus described our invention, what we claim as new and desire to secure by Letters Patent is:

1. A process of decarburizing silicon steel sheet or strip containing from 0.05% to 4% silicon

which comprises open annealing said sheet or strip at a temperature substantially within the range of 1350 to 1650 degrees F., in an atmosphere predominantly of hydrogen and containing water vapor substantially within the range of two to thirty-five per cent.

2. A process of decarburizing silicon steel sheet or strip containing silicon between substantially 0.05% and substantially 4% and containing originally not substantially less than 0.02 per cent carbon, and having a gauge not substantially greater than 0.025 inch, which comprises heating the sheet or strip at a temperature substantially within the range of 1350 to 1650 degrees F. in a non-oxidizing atmosphere predominantly of hydrogen and containing substantially four to thirty-five per cent water vapor in an open anneal to reduce the carbon content of said silicon steel to a value not greater than 0.01 per cent, but not exceeding 30 minutes in duration.

3. A process of producing silicon steel containing substantially 0.05% to 4% silicon which comprises hot rolling the silicon steel to an intermediate gauge, pickling it, cold rolling it to sheet gauge, and open annealing it so that for at least a portion of the cycle it is at a temperature substantially between 1400 and 1600 degrees F. in a reducing atmosphere containing water vapor in an amount substantially between 4 and 35 per cent, whereby both to decarburize the steel and to develop its magnetic characteristics.

4. A process of producing decarburized silicon steel containing substantially between 0.05% and 4% silicon which comprises hot rolling silicon steel to an intermediate gauge, pickling it, cold rolling it to gauge, and open annealing it so that for at least a portion of the cycle it is at a temperature substantially between 1400 and 1600 degrees F. in an atmosphere predominantly of hydrogen but containing water vapor in an amount substantially between four and thirty-five per cent, the initial carbon content of said silicon steel being substantially within the range of 0.02 and 0.06 per cent, and said open annealing being carried on for a sufficient length of time to develop the magnetic characteristics of the material and to reduce the carbon content of said silicon steel to a value not substantially greater than 0.01 per cent, the final gauge of said material being not substantially greater than 0.025 inch and the time duration of said treatment lying substantially between two and fourteen minutes.

5. A process of producing decarburized silicon steel containing from 0.05% to 4% silicon which comprises hot rolling it to an intermediate gauge, pickling it, cold rolling it to within five to ten per cent of final gauge, open annealing it at a temperature substantially between 1400 and 1600 degrees F. in a reducing atmosphere containing water vapor substantially between two and thirty-five per cent whereby to decarburize the silicon steel, then cold rolling it to final gauge and finally open annealing it at a temperature not substantially less than 1400 degrees F., whereby to develop its magnetic characteristics, the final gauge of said material being not substantially greater than 0.025 inch, the initial carbon content of said material lying substantially within the range of 0.02 and 0.06 per cent and the final carbon content of said material being not substantially greater than 0.015 per cent.

6. A process of producing silicon steel containing substantially between 0.05% and 4% silicon, characterized by high permeability in the rolling

direction, and low carbon content, which comprises hot rolling the material to a thickness substantially within the range of 0.07 to 0.15 inch, cold rolling the material to give it a reduction of substantially between 60 and 85 per cent while controlling the temperature so as to produce in the metal in addition to cold-rolling orientation an incipient twinned condition of the crystals, open annealing the material so that for at least a portion of the cycle it is at a temperature substantially between 1400 and 1600 degrees F. in an atmosphere predominantly of hydrogen but containing water vapor in an amount substantially between four and thirty-five per cent, whereby both to reduce the carbon content and to cause the twinned condition of the crystals to grow by accretion, again cold rolling the material with a reduction of substantially between 50 and 85 per cent while controlling the temperature as before, and finally open annealing the material whereby the crystal orientation in the finished material is predominantly of the twin-derivative type.

7. A process of producing silicon steel containing substantially 0.05% to 4% silicon, characterized by high permeability and low core loss in the rolling direction, and low carbon content, which comprises hot rolling the material to a gauge substantially within the range of 0.07 and 0.15 inch, cold rolling the material to give it a reduction of substantially between 60 and 85 per cent while controlling the temperature so as to produce in the metal in addition to cold-rolling orientation an incipient twinned condition of the crystals, open annealing the material so that at least for a portion of the cycle it is at a temperature substantially between 1400 and 1600 degrees F. in a reducing atmosphere containing water vapor in an amount substantially between four and thirty-five per cent whereby both to reduce the carbon content and to cause the twinned condition of the crystals to grow by accretion, again cold rolling the material with a reduction of substantially between 50 and 85 per cent while controlling the temperature as before, and finally box annealing the material in an atmosphere predominantly of hydrogen whereby the crystal orientation in the finished material is predominantly of the twin-derivative type, the initial carbon content of said silicon steel being of the order of 0.02 and 0.06 per cent and the final carbon content of said silicon steel being not substantially greater than 0.008 per cent.

8. A process of producing silicon steel containing substantially 0.05% to 4% silicon, characterized by high permeability and low core loss in the rolling direction, and low carbon content, which comprises hot rolling the material to a gauge substantially within the range of 0.07 to 0.15 inch, cold rolling the material to give it a reduction of substantially between 60 and 85 per cent while controlling the temperature so as to produce in the metal in addition to cold-rolling orientation an incipient twinned condition of the crystals, open annealing the material so that for at least a portion of the cycle it is at a tempera-

ture substantially between 1350 and 1650 degrees F. in an atmosphere predominantly of hydrogen but containing water vapor in an amount substantially between two and thirty-five per cent, whereby both to reduce the carbon content and to cause the twinned condition of the crystals to grow by accretion, again cold rolling the material with a reduction of substantially between 50 and 85 per cent while controlling the temperature as before, again open annealing the material at a temperature substantially between 1350 and 1650 degrees F. in an atmosphere predominantly of hydrogen but containing water vapor in an amount substantially between two and thirty-five per cent, whereby to further reduce the carbon content, and finally box annealing the material predominantly in hydrogen, the final carbon content of said silicon steel being not substantially greater than 0.008 per cent and the crystal orientation in the finished material being predominantly of the twin-derivative type.

9. A process as set forth in claim 8, in which the material is box annealed following the hot rolling, in the presence of its hot-mill scale whereby to effect an initial decarburization.

10. A process of producing silicon steel sheet or strip containing substantially 0.05% to 4% silicon, which comprises hot rolling silicon steel to an intermediate gauge, box annealing said silicon steel in the presence of the hot-mill scale, resulting from said hot rolling so as to lower the carbon content of said steel, afterward further reducing the steel by rolling to a lighter gauge, and open annealing the steel in an atmosphere of reducing gas containing substantially two to thirty-five per cent water vapor at a temperature substantially between 1350° and 1650° F. so as to lower the carbon content still further.

11. A process of making low carbon ferrous materials which comprises producing a ferrous material containing at least 0.05 to substantially 4 per cent silicon, reducing said material to a gauge not substantially greater than 0.025 inch, and open annealing the reduced material at a temperature substantially between 1350° and 1650° F. in an atmosphere of reducing gas containing at least substantially two per cent water vapor so as to lower the carbon content thereof.

12. A process of producing decarburized silicon steel containing substantially 0.05% to 4% silicon, including the steps of reducing silicon steel to sheet-like form and annealing said steel to impart desired magnetic properties thereto and which comprises subjecting the material to a heat treatment within the range of 1350 degrees to 1650 degrees F. in a reducing atmosphere containing water vapor substantially within the range of 2 per cent to 35 per cent, at a stage of the process at which the gauge of the material is substantially within the range of 0.012 to 0.025 inch, the duration of said annealing treatment being from substantially two to substantially fourteen minutes.

VICTOR W. CARPENTER.  
JOHN M. JACKSON.